

1

3,168,380  
COLUMBIUM BASE ALLOYS

Elihu F. Bradley, West Hartford, Conn., and John J. Rausch, Evanston, Joseph B. McAndrew, Chicago, and Charles R. Simcoe, Evergreen Park, Ill., assignors, by direct and mesne assignments, to United Aircraft Corporation, Hartford, Conn., a corporation of Delaware  
No Drawing. Filed Nov. 3, 1961, Ser. No. 149,879

6 Claims. (Cl. 29—194)

This invention relates to novel columbium base alloys and more particularly to an alloy of columbium comprising an improved columbium aluminide compound that is resistant to oxidation at all temperatures up through 2550° F. and to methods of making and using such alloys.

The principal limitation in gas turbine technology today is the maximum turbine inlet temperature. The turbine inlet temperature is in turn limited by the temperature that the turbine vanes and blades are able to withstand without danger of failure. The best available high temperature alloys in the prior art have been nickel and cobalt base superalloys, but critical structural components such as turbine vanes and blades constructed from such alloys are limited to maximum operating temperatures of between 1600° and 1900° F.

Among the technically most important physical qualities of columbium as an alloy base are its high melting temperature (4380° F.) and its low neutron-capture cross-section. Columbium is, therefore, potentially useful for fast aircraft and space flight vehicles and in nuclear reactors.

For many years it has been generally known that high-temperature strength properties of metals are closely related to their melting points. Thus, metals having a high melting point also tend to have high-temperature strength potentials.

The need for structural materials for service at temperatures in excess of those attainable with present materials of construction has stimulated interest in the refractory metals. Until about 1957 molybdenum was considered the chief prospect for such uses. However, at the high temperature service conditions needed, molybdenum oxidizes at a catastrophic rate, principally because molybdenum oxide is volatile at elevated temperatures. Because of the great problems encountered in attempting to coat molybdenum, interest has recently shifted to columbium as an alloy base for high-temperature service.

Columbium is inherently a soft, ductile, readily-fabricable material. Although its melting temperature is about 4380° F., pure columbium becomes too weak for structural use at temperatures above 1200° F. Columbium is a very reactive metal in that it dissolves large quantities of oxygen, and probably also nitrogen, on exposure to atmospheres containing even small amounts of these elements at modest temperatures.

Although columbium suffers from oxidation, its oxide does not volatize, and it is thus potentially possible to localize oxygen attack on columbium by coating the metal. Further advantages offered by columbium base alloys as compared with molybdenum base alloys are that columbium base alloys are relatively more ductile and workable at low temperatures and columbium has a lower density than molybdenum.

Until recent years, estimated ore reserves of columbium were so small that there was only a mild interest in columbium base alloys. With the discovery of substantial ore bodies, however, the potential availability of columbium is so much greater than formerly that scarcity can no longer be considered a restriction on its use.

We have discovered and disclosed in our copending application Serial No. 150,628, filed November 7, 1961, that

2

the compound columbium aluminide when applied to columbium base alloys by an electrodeposition process gives excellent oxidation resistance to columbium and columbium base alloys in the temperature range 2100° to 2550° F. The electrodeposition coating process there disclosed for coating aluminum on columbium base alloys to provide the compound columbium aluminide as a coating provides excellent control of the uniformity of the coating, particularly at edges and corners of the piece being coated. This coating process is thus effective to clad columbium base alloy articles of even intricate shapes with a uniform protective coating.

The coatings and processes for applying these coatings as disclosed in our copending application Serial No. 150,628, filed November 7, 1961, are particularly effective in providing an oxidation resistant protective coating to columbium base alloys of the type disclosed in copending application Serial No. 358,972, filed April 6, 1964.

In testing columbium base alloy articles that had been coated with columbium aluminide as disclosed in our copending application Serial No. 150,628, filed November 7, 1961, we learned that although the columbium aluminide coating provided excellent oxidation resistance for the columbium base alloys at temperatures in the range 2100° to 2500° F., erratic results were obtained at temperatures below 2100° F. For example, specimens of columbium base alloys coated with columbium aluminide that were tested at a temperature of 1830° F. showed a maximum effective life of only about eight (8) hours.

When these specimens were first subjected to prior exposure at higher temperatures, such as 2200° to 2400° F., and subsequently exposed at 1830° F., catastrophic oxidation ensued and powdering of the coating occurred within fifteen (15) minutes.

The occurrence of this phenomenon was at first attributed to the rearrangement that occurs in the coating during the early stages of oxidation and diffusion of the coating into the base metal of the alloy. To check this theory, coated samples of columbium base alloys were diffused in a vacuum at 1800° F. for four (4) hours prior to exposure in air. This diffusion treatment however, had no apparent effect in retarding the tendency for the coating to powder at low temperatures. The phenomenon was accordingly ascribed to an inherent property of columbium aluminide, and the general oxidation behavior of this compound was then examined.

The compound columbium aluminide ( $CbAl_3$ ) when oxidized at 1200° to 1400° F. undergoes a disintegration in which the bulk material is converted to a fine gray powder in a manner analogous to the behavior of  $MoSi_2$  at low temperatures as originally reported by E. Fitzer, in Molybdandisilizid als Hochtemperaturwerkstoff, Plansee Proc., 1955, Pergamon Press, London, 1956. At 1200° to 1400° F., powdering occurs within two to three hours. At 1000° F., an incubation period of about 150 hours is required, after which powdering progresses at a rapid rate.

Oxidation in the temperature range 1400° to 1800° F. has not been examined thoroughly; however, it appears that at these temperatures a combination of disintegration by powdering and normal scaling occurs.

As disclosed in our copending application Serial No. 150,628, filed Nov. 7, 1961, oxidation of columbium aluminide within the temperature range 2100° to 2550° F. is at a minimum, and is sufficient to provide excellent oxidation resistance when used as a coating on columbium base alloys for a period of 100 hours or more. After this initial period of good oxidation resistance there is a transition to a more rapid oxidation rate in the 2100° to 2550° F. range.

At 1400° F. oxidation proceeds at a low rate until

the onset of powdering which begins after two to three hours of exposure. Thereafter, an abnormally large weight gain is observed, that, after 40 hours, corresponds to an accession of 6.2 mols of oxygen per mol of  $\text{CbAl}_3$ .

At high temperatures the scale formed on columbium aluminide ( $\text{CbAl}_3$ ) consists of a mixture of  $\alpha\text{-Al}_2\text{O}_3$  and the H-allotrope of  $\text{Cb}_2\text{O}_5$ . To determine if the powdering at low temperatures was associated with an allotropic transformation in columbium aluminide ( $\text{CbAl}_3$ ), specimens of this material were heated in a vacuum for 300 hours at temperatures varying between 800° and 1200° F. No evidence of powdering was observed. Although these experiments do not exclude the possibility of a low-temperature allotrope of  $\text{CbAl}_3$  being stabilized by oxygen, they do confirm an essential relationship of environment to the disintegration observed.

It was then decided to study the effect that alloying additions to the compound columbium aluminide ( $\text{CbAl}_3$ ) might have in helping to overcome the tendency of  $\text{CbAl}_3$  to powder at low temperatures.

Many alloy additions to  $\text{CbAl}_3$  were made and tested. Finally, we discovered that the addition of small amounts of silicon to columbium aluminide would have a dramatic and remarkably beneficial effect in improving the oxidation resistance of columbium aluminide at all temperatures up to 2550° F.

In view of the foregoing description, it is a primary object of this invention to provide an oxidation resistant columbium aluminide compound that has excellent resistance to oxidation at all temperatures up through 2550° F.

Additional objects of this invention are to provide a columbium aluminide compound for coating columbium and columbium base alloys that will provide excellent oxidation resistance for the alloys at all temperatures up through 2550° F., that when used for a coating will be impermeable to gases, that will provide a low rate of interdiffusion between the coating and the base metal, and that will be relatively ductile at all temperatures.

A further object of this invention is to provide a novel columbium aluminide compound for coating columbium and columbium base alloys that comprises columbium aluminide and from about 3 to 10 atomic percent of silicon to improve the oxidation resistance of the columbium aluminide at all temperatures up through 2550° F., and particularly to dramatically and remarkably improve the oxidation resistance of columbium aluminide in the lower temperature range of from 1200° to 2000° F.

The foregoing and other objects are realized by the alloys of this invention that contain as essential ingredients columbium aluminide that is made up of about 75 atomic percent aluminum, balance columbium, to which is added about 3 to 10 atomic percent silicon.

Although the amounts of silicon to be added to columbium aluminide to form the alloys of this invention may vary from between about 3 and 10 atomic percent silicon, the amounts are usually between about 4 and 7 atomic percent, and are preferably between about 5 and 6 atomic percent silicon.

The novel alloys or compounds of this invention can be prepared by using known melting and casting techniques. To ensure homogeneity, it may be desirable to use multiple melting. Individual melts can be melt-cast together, and the melt may be permitted to cool and solidify into a pre-determined shape.

In operation the melting can be achieved by either an induction-type furnace or an arc furnace using either consumable or non-consumable electrodes. An arc melting furnace using a chilled copper crucible has been used advantageously.

Regardless of the type of furnace used, great care must be taken in the melting and casting operation to protect the molten metal from normal atmospheric contamination by oxygen, nitrogen, and other gases that may be present. This problem can be avoided by conducting the melting operation in a controlled atmosphere.

In preparing the metals for the charge almost any appropriate form of the metals may be used, such as shot, granular, powder, or wire. Ideally, the metals should be of the highest purity commercially obtainable. In the examples set forth below 10-gram melts were prepared and tested for oxidation at various temperatures as described in the examples. Weight gain was measured as a function of time.

The behavior of columbium aluminide ( $\text{CbAl}_3$ ) at a number of temperatures below 2000° F. has already been described. It may be helpful, however, to describe the oxidation behavior of columbium aluminide ( $\text{CbAl}_3$ ) when in the pure form at temperatures of 2000° F. and 2400° F. The oxidation behavior of pure columbium aluminide ( $\text{CbAl}_3$ ) at these temperatures may then be compared with the test results obtained from the examples described below.

At 2000° F. columbium aluminide ( $\text{CbAl}_3$ ) displays good oxidation resistance for approximately 100 hours, it then undergoes a transition to an increased rate of oxidation. At the end of 100 hours of exposure columbium aluminide ( $\text{CbAl}_3$ ) at 2000° F. will show a weight gain of approximately 10 mg./cm.<sup>2</sup>.

At 2400° F. the oxidation of columbium aluminide ( $\text{CbAl}_3$ ) proceeds at a more rapid rate, and the compound will experience a weight gain of about 20 mg./cm.<sup>2</sup> after 30 hours of exposure.

For a clearer understanding of the invention, specific examples of the invention are given below. These examples are merely illustrative and are not to be understood as limiting the scope and underlying principles of the invention.

#### EXAMPLE I

A mixture of 22.5 atomic percent of columbium, 72.5 atomic percent of aluminum, and 5 atomic percent of silicon was introduced as a charge into a water-cooled, copper crucible of a non-consumable, electrode type melting furnace using tungsten electrodes. Prior to melting the furnace chamber was evacuated four (4) times and then back-filled with argon to provide a sufficiently inert air-free controlled atmosphere. Each charge was melted a minimum of two (2) times, with the total number of melts needed for homogeneity being determined by operator observation. When the charge had been melted for the last time, the furnace was turned off and the melt was allowed to cool in the argon atmosphere, discharged from the crucible, and tested as described below.

All melts were prepared as 10-gram melts and the testing procedure that was used for this example was also used for all the other examples given.

As oxidation resistance is the primary object of this invention, the examples given were tested for oxidation resistance only, and not for other alloy characteristics, since it is known that columbium aluminide has characteristics that make it satisfactory in other respects as a coating for columbium and columbium base alloys.

For oxidation tests specimens were exposed to a static air-atmosphere at the temperatures and for the times described below. Specimens were prepared by grinding to a uniform finish with an aluminum oxide grit abrasive. After carefully weighing and measuring all critical components, the specimens were exposed in pre-fired porcelain crucibles in such a manner that the maximum surface exposure was achieved. After exposure each specimen was evaluated by measuring weight gain and by visual observation of the specimens.

The specimen of this example was exposed for 140 hours at 2000° F. and showed no appreciable weight gain at the end of this period. The specimen after exposure had a dark grey, tightly bound oxide film that formed during the initial stage of oxidation and did not change appreciably even after 140 hours. The oxidation behavior of the columbium aluminide ( $\text{CbAl}_3$ ) plus 5 atomic percent silicon specimen of this example regis-

tered a significant improvement over the oxidation behavior of pure columbium aluminide ( $\text{CbAl}_3$ ) at 2000° F. Pure columbium aluminide ( $\text{CbAl}_3$ ) begins to oxidize fairly rapidly after 100 hours of exposure at 2000° F.

Another specimen of this example was exposed to oxidation in air for 145 hours at 2400° F. After 145 hours of exposure the compound showed no appreciable weight change and maintained virtually the same high oxidation resistance that it had shown at 2000° F.

The first specimen described above after prior exposure at 2000° F. for 145 hours was exposed at 1800° F. for 40 hours with no detectable weight gain and was then exposed at 1600° F. for 40 hours, again, with no detectable weight gain. Similarly, the specimen above, that was exposed at 2400° F. for 145 hours was exposed at 1800° F. for 40 hours after the prior exposure, and no detectable weight gain was registered. This specimen was then exposed at 1600° F. for 40 additional hours; again, no detectable weight gain was noted.

Another specimen of this example was then exposed, without prior high-temperature treatment at 1200° F. for 83 hours. This specimen showed no powdering or change in weight after this exposure.

From these test results it is apparent that the addition of relatively small amounts of silicon to columbium aluminide ( $\text{CbAl}_3$ ) are remarkably beneficial in improving the oxidation resistance of columbium aluminide ( $\text{CbAl}_3$ ) at all temperatures.

#### EXAMPLE II

A 10-gram melt of columbium aluminide ( $\text{CbAl}_3$ ) containing two (2) atomic percent silicon, with each atom of silicon replacing one atom of columbium and three (3) atoms of aluminum respectively, was prepared as described in Example I. Static oxidation tests of this specimen were performed at 1200°, 2000°, and 2400° F. After 10 hours' exposure at 1200° F. this specimen showed a weight gain of 40 mg./cm.<sup>2</sup>; after 10 hours' exposure at 2000° F., it showed a weight gain of 8 mg./cm.<sup>2</sup>, and after 170 hours' exposure at 2400° F., it showed a weight gain of 21 mg./cm.<sup>2</sup>. This specimen was thus obviously unsatisfactory in the lower temperature ranges.

#### EXAMPLES III THRU VIII

10-gram melts of columbium aluminide ( $\text{CbAl}_3$ ) containing, respectively, 0.5, 1, 3, 4, 6, and 8 atomic percent silicon were prepared as Examples III through VIII respectively, as described in Examples I and II. These examples were then tested for oxidation behavior in the same manner as the tests set forth in Example I. The results of these tests are presented in Table I.

Table I

| Example No. | Percentage of silicon in atomic percent | Testing Temp. of 1,200° F. |                                  | Testing Temp. of 2,000° F. |                                  | Testing Temp. of 2,400° F. |                                  |
|-------------|-----------------------------------------|----------------------------|----------------------------------|----------------------------|----------------------------------|----------------------------|----------------------------------|
|             |                                         | Exposure to Air in Hours   | Wt. gain in mg./cm. <sup>2</sup> | Exposure to Air in Hours   | Wt. gain in mg./cm. <sup>2</sup> | Exposure to Air in Hours   | Wt. gain in mg./cm. <sup>2</sup> |
| III         | 0.5% Si                                 |                            |                                  | 170                        | 155                              | 40                         | 27                               |
| IV          | 1% Si                                   |                            |                                  | 170                        | 42                               | 40                         | 51                               |
| V           | 2% Si                                   | 10                         | 40                               | 10                         | 8                                | 170                        | 21                               |
| V           | 3% Si                                   | 380                        | about 1                          | 320                        | about 5                          | 170                        | about 17                         |
| VI          | 4% Si                                   | 190                        | 0                                | 170                        | about 4                          | 170                        | about 22                         |
| I           | 5% Si                                   | 83                         | 0                                | 145                        | about 1                          | 145                        | about 1                          |
| VII         | 6% Si                                   | 190                        | about 1                          | 170                        | about 9                          | 170                        | about 19                         |
| VIII        | 8% Si                                   | 190                        | about 2                          | 170                        | about 12                         | 150                        | about 17                         |

From the results of the foregoing tests, it is known that, at all temperatures, a minimum silicon concentration is required to eliminate the destructive powdering reaction and rapid oxidation of columbium aluminide ( $\text{CbAl}_3$ ). Slightly beyond this minimum value the oxidation rate becomes lowest at each temperature. Higher silicon concentrations then produce an increase in the rate of oxidation; however, the oxidation rate of each of the higher silicon

tions and examples which do not sacrifice their chief advantages.

70 What is claimed is:

1. A high-temperature oxidation resistant composition of matter consisting of aluminum and columbium in an atomic ratio of about 3 to 1 and from 3 to 10 atomic percent of silicon based on the sum total of atoms in the composition.

alloys tested is quite acceptable at all temperatures. The minimum silicon concentration that will prevent powdering appears to be temperature dependent but occurs in the range of two (2) to three (3) atomic percent silicon.

5 Microscopic examination of the columbium aluminide-silicon compounds reveals the presence of second phase located at the columbium aluminide ( $\text{CbAl}_3$ ) grain boundaries. The grain boundary constituent has a eutectic microstructure and becomes continuous at about the composition columbium aluminide plus three (3) atomic percent silicon. Increased silicon concentration increases the quantity of the grain boundary material.

10 In summary the compound columbium aluminide ( $\text{CbAl}_3$ ) applied by the electrodeposition of molten aluminum onto a columbium substrate has shown very promising results. The compound columbium aluminide when coated on columbium or columbium base alloys drastically improves the oxidation resistance of the base metal at temperatures in the range 2100° to 2550° F.

15 At temperatures below 2100° F., however, the columbium aluminide coating exhibits poor resistance to oxidation. This result was traced to the inherent oxidation behavior of columbium aluminide at these temperatures. At low temperatures (1200°-1400° F.), columbium aluminide undergoes a transition in which the bulk material is converted to a fine gray powder within two to three hours. At slightly higher temperatures (1400°-1800° F.) oxidation is rapid and occurs by a combination of disintegration by powdering and normal scaling.

20 To overcome the low-temperature deficiencies of columbium aluminide the effect of alloying additions was studied. The discovery was made that silicon in concentrations greater than about (3) atomic percent, provides a dramatic and unexpected beneficial result in preventing the catastrophic low temperature attack of oxygen on columbium aluminide ( $\text{CbAl}_3$ ). It has also been discovered that the addition of 5 atomic percent of silicon to columbium aluminide reduces the 2400° F. scaling rate of this compound by a factor of twenty (20). This latter result was also unexpected and unusually beneficial.

25 The alloys of this invention comprising columbium aluminide and at least about 3 atomic percent silicon because they are oxidation resistant over all temperature ranges up through 2550° F., offer unusually high promise as coatings for protecting columbium and columbium base alloys from oxidation at high temperatures.

30 The present invention in its broader aspects is not limited to the specific compositions and examples described, but also includes within the scope of the accompanying claims any departures made from such composi-

2. A high-temperature oxidation resistant composition of matter consisting of aluminum and columbium in an atomic ratio of about 3 to 1 and from 4 to 7 atomic percent of silicon based on the sum total of atoms in the composition.

3. A high-temperature oxidation resistant composition of matter consisting of aluminum and columbium in an atomic ratio of about 3 to 1 and about 5 atomic percent of silicon based on the sum total of atoms in the composition.

4. A high-temperature oxidation resistant columbium base alloy containing at least 40 per cent by weight of columbium and having a coating comprising a composition of matter consisting of aluminum and columbium in an atomic ratio of about 3 to 1 and from 3 to 10 atomic per cent of silicon based on the sum total of atoms in the composition.

5. A high-temperature oxidation resistant columbium base alloy containing at least 40 percent by weight of columbium and having a coating comprising a composition of matter consisting of aluminum and columbium in an atomic ratio of about 3 to 1 and from 4 to 7 atomic per-

cent of silicon based on the sum total of atoms in the composition.

6. A high-temperature oxidation resistant columbium base alloy containing at least 40 percent by weight of columbium and having a coating comprising a composition of matter consisting of aluminum and columbium in an atomic ratio of about 3 to 1 and about 5 atomic percent of silicon based on the sum total of atoms in the composition.

10

## References Cited in the file of this patent

## UNITED STATES PATENTS

3,102,044 Joseph \_\_\_\_\_ Aug. 27, 1963

## FOREIGN PATENTS

15 1,099,179 Germany \_\_\_\_\_ Feb. 9, 1961

## OTHER REFERENCES

20 Carlson: "Oxidation Resistance of Aluminum Dip Coated (Aldico) Columbium Alloys," Columbium Metallurgy, vol. 10, Metallurgical Society of A.I.M.E., Interscience Publishers, New York 1, N. Y. (from papers presented June 9-10, 1960); pp. 119-137.